

## UNITED STATES PATENT OFFICE.

FRITZ PETERHAUSER, OF RIEHEN, NEAR BASEL, SWITZERLAND, ASSIGNOR TO THE FIRM DURAND & HUGUENIN S. A., OF BASEL, SWITZERLAND.

## PRODUCTION OF FAST DYEINGS.

No Drawing. Application filed March 12, 1925, Serial No. 15,136, and in Germany March 20, 1924.

According to U. S. Letters Patent application Ser. No. 653,567, filed July 24, 1923, fast dyeings are produced on fibres or other substrata by impregnating the latter with 5 solutions of ester salts of vat dyestuffs, such as are obtained according to the process of U. S. Letters Patent No. 1,448,251, and by developing afterwards the dyeing, by way of re-formation of the parent vat dyestuff, 10 with the assistance of a suitable oxidizing agent. In above mentioned Letters Patent application Ser. No. 653,567, it has been stated that these ester salts have for the most part no affinity to the material to be dyed. With reference to the animal fibre, this statement has been modified as in the same Letters Patent application further down it has been mentioned that these ester salts fix themselves on the animal fibre from 15 a weak acid bath and at a higher temperature.

It has now further been found that various cellulosic fibres, especially cotton, mercerized cotton, viscose and the like acquire 20 an essentially enhanced receptivity for these ester salts when there is added to the dye-bath a salt which is capable of lessening the solubility of the ester-salt in water and thus increases the proportion of the ester-salt 25 taken up by the fibre, so that in the subsequent development in the oxidation bath, much deeper dyeings can be obtained than without this addition of salt, a fact which greatly enhances the dyeing. Salts which 30 are suitable for this purpose are for example common salt, Glauber salt etc.

The improved process may be explained by the following example:

In a bath containing 6.6 grs. of the sodium 35 salt of the leuco indigo sulphuric acid ester, obtained according to Example I of said U. S. Letters Patent No. 1,448,251, 6.6 grs. of nitrite and 33 grs. of Glauber salt, viscose is impregnated at ordinary temperature

during about  $\frac{1}{4}$  of an hour. Then wring 45 the goods, and without rinsing develop in a bath which contains per 100 grs. of bath, 2 grs. of sulphuric acid at a strength of 96%, and to which the same quantity of salt has been added as in the case of the first bath. 50 Then rinse and dry. Thus a deep dyeing fast to rubbing is obtained, which is much deeper than the one which could have been obtained without the addition of salt to the dye bath.

Instead of viscose, cotton or mercerized cotton can be dyed in the same way.

The effect of this addition of salt seems to vary on the different fibres. On viscose the effect is especially strong. On weavings 60 with different threads and the like, dyeing effects of different intensity can also be produced according to this process.

Obviously the oxidation will be effected in a second bath with iron chloride, nitrite 65 and sulphuric acid etc. as stated in the cited U. S. Letters Patent application Ser. No. 653,567.

## What I claim is:

1. A process for producing fast dyeings 70 by means of ester salts of vat-dyestuffs resulting from their leuco-compound polybasic acid esters, consisting in adding to the dye bath a solubility lessening salt capable of increasing the absorption power of the fibre 75 for the vat dyestuff ester salts, for the purpose of producing deeper dyeings.

2. A process for producing fast dyeings 80 by means of ester salts of vat-dyestuffs resulting from their leuco-compound polybasic acid esters, consisting in adding Glauber salt to the dye bath so as to increase the absorption power of the fibre for the vat-dyestuff ester salts, for the purpose of producing deeper dyeings.

In witness whereof I have hereunto signed my name this 28th day of February, 1925.

FRITZ PETERHAUSER.